



US007344813B2

(12) **United States Patent**  
**Sweeney et al.**

(10) **Patent No.:** **US 7,344,813 B2**  
(b5) **Date of Patent:** **Mar. 18, 2008**

|      |                                                                                                                                                                                                                                                                                                                                                                                       |             |         |                            |
|------|---------------------------------------------------------------------------------------------------------------------------------------------------------------------------------------------------------------------------------------------------------------------------------------------------------------------------------------------------------------------------------------|-------------|---------|----------------------------|
| (54) | <b>EMULSION AGGREGATION TONER HAVING GLOSS ENHANCEMENT AND TONER RELEASE</b>                                                                                                                                                                                                                                                                                                          | 4,338,390 A | 7/1982  | Lu                         |
| (75) | Inventors: <b>Maura A. Sweeney</b> , Irondequoit, NY (US); <b>Grazyna E. Kmiecik-Lawrynowicz</b> , Fairport, NY (US); <b>Matthew L. Fabrizio</b> , Rochester, NY (US); <b>Robert D. Bayley</b> , Fairport, NY (US); <b>Karen A. Moffat</b> , Brantford (CA); <b>David J. Sanders</b> , Oakville (CA); <b>Enno E. Agur</b> , Toronto (CA); <b>Daryl W. Vanbesien</b> , Burlington (CA) | 4,935,326 A | 6/1990  | Creatura et al.            |
|      |                                                                                                                                                                                                                                                                                                                                                                                       | 4,937,166 A | 6/1990  | Creatura et al.            |
|      |                                                                                                                                                                                                                                                                                                                                                                                       | 5,278,020 A | 1/1994  | Grushkin et al.            |
|      |                                                                                                                                                                                                                                                                                                                                                                                       | 5,290,654 A | 3/1994  | Sacripante et al.          |
|      |                                                                                                                                                                                                                                                                                                                                                                                       | 5,308,734 A | 5/1994  | Sacripante et al.          |
|      |                                                                                                                                                                                                                                                                                                                                                                                       | 5,344,738 A | 9/1994  | Kmiecik-Lawrynowicz et al. |
|      |                                                                                                                                                                                                                                                                                                                                                                                       | 5,346,797 A | 9/1994  | Kmiecik-Lawrynowicz et al. |
|      |                                                                                                                                                                                                                                                                                                                                                                                       | 5,348,832 A | 9/1994  | Sacripante et al.          |
|      |                                                                                                                                                                                                                                                                                                                                                                                       | 5,364,729 A | 11/1994 | Kmiecik-Lawrynowicz et al. |
|      |                                                                                                                                                                                                                                                                                                                                                                                       | 5,366,841 A | 11/1994 | Patel et al.               |
|      |                                                                                                                                                                                                                                                                                                                                                                                       | 5,370,963 A | 12/1994 | Patel et al.               |
|      |                                                                                                                                                                                                                                                                                                                                                                                       | 5,403,693 A | 4/1995  | Patel et al.               |
|      |                                                                                                                                                                                                                                                                                                                                                                                       | 5,405,728 A | 4/1995  | Hopper et al.              |
|      |                                                                                                                                                                                                                                                                                                                                                                                       | 5,418,108 A | 5/1995  | Kmiecik-Lawrynowicz et al. |
|      |                                                                                                                                                                                                                                                                                                                                                                                       | 5,462,828 A | 10/1995 | Moffat et al.              |
|      |                                                                                                                                                                                                                                                                                                                                                                                       | 5,496,676 A | 3/1996  | Croucher et al.            |
|      |                                                                                                                                                                                                                                                                                                                                                                                       | 5,501,935 A | 3/1996  | Patel et al.               |
|      |                                                                                                                                                                                                                                                                                                                                                                                       | 5,527,658 A | 6/1996  | Hopper et al.              |
|      |                                                                                                                                                                                                                                                                                                                                                                                       | 5,585,215 A | 12/1996 | Ong et al.                 |
|      |                                                                                                                                                                                                                                                                                                                                                                                       | 5,650,255 A | 7/1997  | Ng et al.                  |
|      |                                                                                                                                                                                                                                                                                                                                                                                       | 5,650,256 A | 7/1997  | Veregin et al.             |
|      |                                                                                                                                                                                                                                                                                                                                                                                       | 5,723,253 A | 3/1998  | Higashino et al.           |
|      |                                                                                                                                                                                                                                                                                                                                                                                       | 5,744,520 A | 4/1998  | Kmiecik-Lawrynowicz et al. |
|      |                                                                                                                                                                                                                                                                                                                                                                                       | 5,747,215 A | 5/1998  | Ong et al.                 |
|      |                                                                                                                                                                                                                                                                                                                                                                                       | 5,763,133 A | 6/1998  | Ong et al.                 |
|      |                                                                                                                                                                                                                                                                                                                                                                                       | 5,766,818 A | 6/1998  | Smith et al.               |

**Related U.S. Application Data**

(63) Continuation-in-part of application No. 10/876,557, filed on Jun. 28, 2004, now Pat. No. 7,179,575.

(Continued)

(51) **Int. Cl.**  
**G03G 9/08** (2006.01)

*Primary Examiner*—John L Goodrow

(52) **U.S. Cl.** ..... **430/108.2; 430/108.3;**  
**430/108.8; 430/137.14**

(74) *Attorney, Agent, or Firm*—Oliff & Berridge, PLC

(58) **Field of Classification Search** ..... **430/108.22,**  
**430/108.1, 108.8, 137.14, 108.3**  
See application file for complete search history.

(57) **ABSTRACT**

(56) **References Cited**

A toner includes particles of a resin, an optional colorant, a first wax and a second wax, where the toner particles are prepared by an emulsion aggregation process. Additional waxes can also be added for different properties.

**U.S. PATENT DOCUMENTS**

3,847,604 A 11/1974 Hagenbach et al.

**17 Claims, 5 Drawing Sheets**



U.S. PATENT DOCUMENTS

|             |         |                            |                   |         |                               |
|-------------|---------|----------------------------|-------------------|---------|-------------------------------|
| 5,804,349 A | 9/1998  | Ong et al.                 | 6,268,099 B1      | 7/2001  | Eguchi et al.                 |
| 5,827,633 A | 10/1998 | Ong et al.                 | 6,500,594 B2      | 12/2002 | Hamano et al.                 |
| 5,840,462 A | 11/1998 | Foucher et al.             | 6,713,918 B2      | 3/2004  | Laing                         |
| 5,853,944 A | 12/1998 | Foucher et al.             | 7,208,252 B2 *    | 4/2007  | Grande et al. .... 430/106.2  |
| 5,869,215 A | 2/1999  | Ong et al.                 | 2002/0051925 A1   | 5/2002  | Matsumura et al.              |
| 5,916,725 A | 6/1999  | Patel et al.               | 2004/0043318 A1   | 3/2004  | Sato et al.                   |
| 5,965,316 A | 10/1999 | Kmiecik-Lawrynowicz et al. | 2004/0137357 A1 * | 7/2004  | Bartel et al. .... 430/137.14 |
| 5,994,020 A | 11/1999 | Patel et al.               | 2006/0057482 A1   | 3/2006  | Yuasa                         |
| 6,120,967 A | 9/2000  | Hopper et al.              |                   |         |                               |

\* cited by examiner



FIG. 1



**FIG. 2**



FIG. 3A



FIG. 3B

## STRIPPING FORCE, LICOWAX TONERS



FIG. 4

## 1

**EMULSION AGGREGATION TONER  
HAVING GLOSS ENHANCEMENT AND  
TONER RELEASE**

**CROSS-REFERENCE TO RELATED  
APPLICATIONS**

This application is a continuation-in-part application of U.S. patent application Ser. No. 10/876,557 filed Jun. 28, 2004, now U.S. Pat. No. 7,179,575 the entire disclosure of which is incorporated herein by reference.

**BACKGROUND**

This present disclosure relates to toners and developers containing the toners for use in forming and developing images of good quality and gloss, and in particular to toners having novel combinations of wax components to provide the desired print quality and high gloss.

Emulsion aggregation toners are excellent toners to use in forming print and/or xerographic images in that the toners can be made to have uniform sizes and in that the toners are environmentally friendly. U.S. patents describing emulsion aggregation toners include, for example, U.S. Pat. Nos. 5,370,963, 5,418,108, 5,290,654, 5,278,020, 5,308,734, 5,344,738, 5,403,693, 5,364,729, 5,346,797, 5,348,832, 5,405,728, 5,366,841, 5,496,676, 5,527,658, 5,585,215, 5,650,255, 5,650,256, 5,501,935, 5,723,253, 5,744,520, 5,763,133, 5,766,818, 5,747,215, 5,827,633, 5,853,944, 5,804,349, 5,840,462, and 5,869,215, the entire disclosures of which are incorporated herein by reference.

Two main types of emulsion aggregation toners are known. First is an emulsion aggregation process that forms acrylate based, e.g., styrene acrylate, toner particles. See, for example, U.S. Pat. No. 6,120,967, incorporated herein by reference in its entirety, as one example of such a process. Second is an emulsion aggregation process that forms polyester, e.g., sodio sulfonated polyester, toner particles. See, for example, U.S. Pat. No. 5,916,725, incorporated herein by reference in its entirety, as one example of such a process.

Emulsion aggregation techniques typically involve the formation of an emulsion latex of the resin particles, which particles have a small size of from, for example, about 5 to about 500 nanometers in diameter, by heating the resin, optionally with solvent if needed, in water, or by making a latex in water using an emulsion polymerization. A colorant dispersion, for example of a pigment dispersed in water, optionally also with additional resin, is separately formed. The colorant dispersion is added to the emulsion latex mixture, and an aggregating agent or complexing agent is then added to form aggregated toner particles. The aggregated toner particles are heated to enable coalescence/fusing, thereby achieving aggregated, fused toner particles.

U.S. Pat. No. 5,462,828 describes a toner composition that includes a styrene/n-butyl acrylate copolymer resin having a number average molecular weight of less than about 5,000, a weight average molecular weight of from about 10,000 to about 40,000 and a molecular weight distribution of greater than 6 that provides excellent gloss and high fix properties at a low fusing temperature.

A principal component in emulsion aggregation toners is a wax. The wax is typically included in the toner particles to provide various properties, such as shape, charging and/or fusing characteristics, gloss, stripping, offset properties, and the like. A problem has been, however, that most waxes

## 2

provides acceptable results only for some of these properties, while providing unacceptable results for other properties.

What is still desired is an improved emulsion aggregation toner that can achieve excellent print quality, particularly gloss, for all colors, while also exhibiting desired properties such as shape, charging and/or fusing characteristics, stripping, offset properties, and the like.

**SUMMARY**

The present disclosure comprises a toner having a novel combination of two or more different waxes that enable the toner to achieve desirable shape, charging, and/or fusing properties not readily attainable by the use of a single wax alone.

In embodiments, the present disclosure provides a toner comprising particles of a resin, an optional colorant, and a combination of at least two different waxes, wherein said toner particles are prepared by an emulsion aggregation process. The combination of waxes can include, for example, combinations of two or more of polyethylene waxes, linear polyethylene waxes, polypropylene waxes, paraffin waxes, Fischer-Tropsch waxes, amide waxes, amine waxes, silicone waxes, carnauba waxes, montan waxes, mercapto waxes, polyester waxes, urethane waxes, microcrystalline waxes, and the like.

In embodiments, the present disclosure also provides methods for making such toners, and developers comprising such toners.

**BRIEF DESCRIPTION OF THE DRAWINGS**

A more complete understanding of the present disclosure can be obtained by reference to the accompanying drawings wherein:

FIG. 1 is a graph relating image gloss to fusing temperature of single wax containing toners described in Comparative Examples 1 to 5.

FIG. 2 is a graph relating stripping force to fusing temperature of single wax containing toners described in Comparative Examples 1 to 5.

FIG. 3a is a graph relating image gloss to fusing temperature of two-component wax containing toners described in Examples 1 to 5, conducted on Lustro Gloss Paper at 0.40 TMA.

FIG. 3b is a graph relating image gloss to fusing temperature of two-component wax containing toners described in Examples 1 to 5, conducted on Lustro Gloss Paper at 1.05 TMA.

FIG. 4 is a graph relating stripping force to fusing temperature of two-component wax containing toners described in Examples 1 to 5, conducted on S-Paper and 1.25 TMA.

**DETAILED DESCRIPTION OF EXEMPLARY  
EMBODIMENTS**

The toner of the present disclosure is comprised of toner particles comprised of at least a latex emulsion polymer resin and a colorant dispersion. The toner particles may also include at least a wax dispersion that comprises a mixture of two or more different waxes. The toner particles can also include a coagulant and a colloidal silica.

Illustrative examples of specific latex for resin, polymer or polymers selected for the toner of the present disclosure include, for example, polyester, poly(styrene-alkyl acrylate),

poly(styrene-1,3-diene), poly(styrene-alkyl methacrylate), poly(styrene-alkyl acrylate-acrylic acid), poly(styrene-1,3-diene-acrylic acid), poly(styrene-alkyl methacrylate-acrylic acid), poly(alkyl methacrylate-alkyl acrylate), poly(alkyl methacrylate-aryl acrylate), poly(aryl methacrylate-alkyl acrylate), poly(alkyl methacrylate-acrylic acid), poly(styrene-alkyl acrylate-acrylonitrile-acrylic acid), poly(styrene-1,3-diene-acrylonitrile-acrylic acid), poly(alkyl acrylate-acrylonitrile-acrylic acid), poly(styrene-butadiene), poly(methylstyrene-butadiene), poly(methyl methacrylate-butadiene), poly(ethyl methacrylate-butadiene), poly(propyl methacrylate-butadiene), poly(butyl methacrylate-butadiene), poly(methyl acrylate-butadiene), poly(ethyl acrylate-butadiene), poly(propyl acrylate-butadiene), poly(butyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), and poly(butyl acrylate-isoprene); poly(styrene-propyl acrylate), poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylic acid), poly(styrene-butyl acrylate-methacrylic acid), poly(styrene-butyl acrylate-acrylonitrile), poly(styrene-butyl acrylate-acrylonitrile-acrylic acid), and other similar polymers.

Illustrative examples of polymer resins selected for the process and particles of the present disclosure include polyesters such as polyethylene-terephthalate, polypropylene-terephthalate, polybutylene-terephthalate, polypentylene-terephthalate, polyhexalene-terephthalate, polyheptadene-terephthalate, polyoctalene-terephthalate, polyethylene-sebacate, polypropylene sebacate, polybutylene-sebacate, polyethylene-adipate, polypropylene-adipate, polybutylene-adipate, polypentylene-adipate, polyhexalene-adipate, polyheptadene-adipate, polyoctalene-adipate, polyethylene-glutarate, polypropylene-glutarate, polybutylene-glutarate, polypentylene-glutarate, polyhexalene-glutarate, polyheptadene-glutarate, polyoctalene-glutarate polyethylene-pimelate, polypropylene-pimelate, polybutylene-pimelate, polypentylene-pimelate, polyhexalene-pimelate, polyheptadene-pimelate, poly(propoxylated bisphenol-fumarate), poly(propoxylated bisphenol-succinate), poly(propoxylated bisphenol-adipate), poly(propoxylated bisphenol-glutarate), SPARTM (Dixie Chemicals), BECKOSOLTM (Reichhold Chemical Inc), ARAKOTETM (Ciba-Geigy Corporation), HETRONTM (Ashland Chemical), PARAPLEXTM (Rohm & Hass), POLYLITETM (Reichhold Chemical Inc), PLAST-HALLTM (Rohm & Hass), CYGALTM (American Cyanamide), ARMCOTM (Armco Composites), ARPOLTM (Ashland Chemical), CELANEXTM (Celanese Eng), RYNITEMTM (DuPont), STYPOLTM (Freeman Chemical Corporation) mixtures thereof and the like, polycarbonates such as LEXANTM (G. E. Plastics), BAYLONTM (Bayer), MAKROLONTM (Mobay), MERLONTM (Mobay), PANLITETM (Teijin Chemical), mixtures thereof and like, polyurethanes such as PELLETHANETM (Dow), ESTANETM (Goodyear), CYTORTM (American Cyanamide), TEXINTM (Mobay), VIBRATHANETM (Uniroyal Chemical), CONATHANETM (Conap Company), mixtures thereof and the like. The resins can also be functionalized, such as sulfonated, if desired.

As the latex emulsion polymer of a toner embodiment, a styrene-alkyl acrylate can be used. Desirably, the styrene-alkyl acrylate is a styrene/n-butyl acrylate copolymer resin, such as a styrene-butyl acrylate beta-carboxyethyl acrylate polymer. As the latex emulsion polymer of an alternative

toner embodiment, a polyester can be used. The polyester can be, for example, a sulfonated polyester, such as a sodio-sulfonated polyester.

The latex polymer may be present in an amount of from about 70 to about 95% by weight of the toner particles (i.e., toner particles exclusive of external additives) on a solids basis, such as from about 75 to about 85% by weight of the toner.

The monomers used in making the selected polymer are not limited, and the monomers utilized may include any one or more of, for example, ethylene, propylene, styrene, acrylates such as methacrylates, butylacrylates,  $\beta$ -carboxy ethyl acrylate ( $\beta$ -CEA), etc., butadiene, isoprene, acrylic acid, methacrylic acid, itaconic acid, acrylonitrile, benzenes such as divinylbenzene, etc., and the like. Known chain transfer agents, for example dodecanethiol or carbon tetrabromide, can be utilized to control the molecular weight properties of the polymer. Any suitable method for forming the latex polymer from the monomers may be used without restriction.

Various suitable colorants can be employed in toners of the present disclosure, including suitable colored pigments, dyes, and mixtures thereof, including carbon black, such as REGAL 330 carbon black, acetylene black, lamp black, aniline black, Chrome Yellow, Zinc Yellow, SICOFAST Yellow, SUNBRITE Yellow, LUNA Yellow, NOVAPERM Yellow, Chrome Orange, BAYPLAST Orange, Cadmium Red, LITHOL Scarlet, HOSTAPERM Red, FANAL PINK, HOSTAPERM Pink, LUPRETON Pink, LITHOL Red, RHODAMINE Lake B, Brilliant Carmine, HELIOGEN Blue, HOSTAPERM Blue, NEOPAN Blue, PV Fast Blue, CINQUASSI Green, HOSTAPERM Green, titanium dioxide, cobalt, nickel, iron powder, SICOPUR 4068 FF, and iron oxides such as MAPICO Black (Columbia) NP608 and NP604 (Northern Pigment), BAYFERROX 8610 (Bayer), M08699 (Mobay), TMB-100 (Magnox), mixtures thereof and the like.

The colorant, such as carbon black, cyan, magenta and/or yellow colorant, is incorporated in an amount sufficient to impart the desired color to the toner. In general, pigment or dye is employed in an amount ranging from about 2% to about 35% by weight of the toner particles on a solids basis, such as from about 5% to about 25% by weight or from about 5 to about 15% by weight.

Of course, as the colorants for each color are different, the amount of colorant present in each type of color toner typically is different. For example, in some embodiments of the present disclosure, a cyan toner may include about 3 to about 11% by weight of colorant (such as Pigment Blue 15:3 from SUN), a magenta toner may include about 3 to about 15% by weight of colorant (such as Pigment Red 122, Pigment Red 185, Pigment Red 238, and/or mixtures thereof), a yellow toner may include about 3 to about 10% by weight of colorant (such as Pigment Yellow 74), and a black toner may include about 3 to about 10% by weight of colorant (such as carbon black).

In addition to the latex polymer binder and the colorant, the toners of the present disclosure also contain a wax dispersion, which wax dispersion comprises a mixture of two or more preferably different waxes. A single wax is typically added to toner formulations in order to improve particular toner properties, such as toner particle shape, presence and amount of wax on the toner particle surface, charging and/or fusing characteristics, gloss, stripping, offset properties, and the like. However, as described above, a problem has been that most waxes provide acceptable results only for some of these properties, while providing

unacceptable or less desirable results for other properties. For example, for styrene-acrylate emulsion/aggregation (E/A) toners, it has been conventional to add linear polyethylene waxes such as the POLYWAX® line of waxes available from Baker Petrolite to the toner composition. The linear polyethylene wax advantageously appears on the surface of the toner particles, and provides good release properties, but provides only fair results in terms of gloss and document offset. However, other waxes, such as high acid montan waxes, carboxylated waxed, amide waxes, and carnauba waxes provide good gloss properties, while providing only fair or poor release and document offset properties.

The present disclosure overcomes the deficiencies of the prior art by providing a hybrid wax system, comprising two or more different waxes. The hybrid wax system can thus provide a range of superior properties, not previously obtainable using a single wax species. Previously most machines used oil on the fuser member as a release system for the electrophotographic process. Recently, with newer chemical toner systems, it has been found that by incorporating wax into the system, particularly into the toner composition, self release from the fuser member without oil was possible. However, experimentation has shown that most conventional waxes, when used alone, do not provide acceptable or desirable results. For example, machines have recently been designed with lower fuser temperatures to improve environmental compliance. As a result, lower melt waxes were required; but the lower melt waxes did not show consistent release properties. It has now been discovered that adding a second or further wax to the system with a slightly higher melt temperature allowed for improved release. Additionally, machine speeds have increased over time, requiring release systems that have good toner release without loss in gloss. The hybrid wax systems of the present disclosure enable excellent release combined with good gloss characteristics.

In embodiments, the hybrid wax system includes two or more waxes. Thus, in embodiments, the hybrid wax system can include two waxes, three waxes, four waxes, or higher numbers of waxes. Additional types of waxes can be added, for example, to achieve different properties or the like. When present, each of the multiple waxes can be present in an effective amount to provide a desired property, rather than being present in only trace or impurity amounts. Thus, for example in a two wax system including waxes A and B, a weight ratio of the respective waxes can range from about 5:95 to about 95:5, such as from about 10:90 to about 90:10, or from about 20:80 to about 80:20. Similarly, in a three wax system, each wax can be present in an amount of at least 5 percent by weight to 90 percent by weight, such as from about 10 to about 80 percent by weight or from about 20 to about 60 percent by weight. Of course, different amounts can be used, as desired.

In embodiments, the hybrid wax system can be provided as a single dispersion of multiple waxes, or as multiple wax dispersions each having one or more waxes. The waxes can be suitably selected from any of the conventionally used toner waxes including, but not limited to, polyolefin waxes, such as polyethylene waxes, including linear polyethylene waxes and branched polyethylene waxes, and polypropylene waxes, including linear polypropylene waxes and branched polypropylene waxes; paraffin waxes; Fischer-Tropsch waxes; amine waxes; silicone waxes; mercapto waxes; polyester waxes; urethane waxes; modified polyolefin waxes (e.g., a carboxylic acid-terminated polyethylene wax or a carboxylic acid-terminated polypropylene wax); amide

waxes, such as aliphatic polar amide functionalized waxes; aliphatic waxes consisting of esters of hydroxylated unsaturated fatty acids; high acid waxes, such as high acid montan waxes; microcrystalline waxes, such as waxes derived from distillation of crude oil; and the like. By "high acid waxes" it is meant a wax material that has a high acid content.

In embodiments, at least one, and more preferably two or all, of the different waxes are crystalline polymeric waxes. By "crystalline polymeric waxes" it is meant that a wax material contains an ordered array of polymer chains within a polymer matrix that can be characterized by a crystalline melting point transition temperature,  $T_m$ . The crystalline melting temperature is the melting temperature of the crystalline domains of a polymer sample. This is in contrast to the glass transition temperature,  $T_g$ , which characterizes the temperature at which polymer chains begin to flow for the amorphous regions within a polymer.

The two or more waxes in the hybrid wax system preferably are different waxes. That is, to achieve the improved properties of the toner compositions, it is preferred that the two or more waxes be different in terms of at least one physical or chemical property, to provide different performance characteristics to the toner composition. Thus, for example, one wax can be selected for its gloss properties, while another wax can be selected for its toner particle shape, presence and amount of wax on the toner particle surface, charging and/or fusing characteristics, stripping, offset properties, or the like. Thus, for example, the waxes can be selected such that a first wax provides improved results in terms of a first property over a second wax, while the second wax provides improved results in terms of a second property over the first wax. The waxes are also preferably selected such that they do not adversely interact or react with each other, to provide inferior or an unusable toner product.

Examples of suitable polyolefin waxes include, but are not limited to, polyethylene waxes and polypropylene waxes. These waxes can be linear or branched, and can be unmodified or modified, e.g., with carboxylic acid groups. Further, the waxes can be crystalline or non-crystalline, although crystalline waxes are preferred, in some embodiments. For example, the polyolefin wax is a crystalline polymeric polyethylene wax. Examples of suitable crystalline polymeric polyethylene waxes include, but are not limited to, the POLYWAX® line of waxes available from Baker Petrolite. Other suitable crystalline polyethylene waxes are also made by and available from Baker Petrolite, as well as other manufacturers. For example, POLYWAX® 725 and/or POLYWAX® 850 are suitable polyethylene (polyolefin) waxes. POLYWAX® 725 and POLYWAX® 850 differ in the molecular weight of the polymer chains. This difference in chain length is also evident in the difference between the crystalline melting point temperatures of these two materials. Baker Petrolite and other manufacturers also produce other polyethylene waxes of lower and higher molecular weight, which can also be used in the hybrid wax system.

In some embodiments where the polyolefin wax is used, the polyolefin wax is not or does not contain a modified polyethylene wax (e.g., a carboxylic acid-terminated polyethylene wax). Thus, in these embodiments, the wax is substantially free or completely free of any modified polyethylene wax, or at least of any crystalline polymeric polyethylene wax that is a carboxylic acid-terminated polyethylene wax. However, such modified waxes can advantageously be used in other embodiments, as desired.

Suitable examples of modified polyolefin waxes, such as carboxylic acid-terminated polyethylene waxes, include, but are not limited to, mixtures of carbon chains with the structure  $\text{CH}_3-(\text{CH}_2)_{n-2}-\text{COOH}$ , where there is a mixture of chain lengths, n, where the average chain length can be in the range of about 16 to about 50, and linear low molecular weight polyethylene, of similar average chain length. Suitable examples of such waxes include, but are not limited to, UNICID® 550 with n approximately equal to 40, and UNICID® 700 with n approximately equal to 50. For example, a particularly suitable crystalline carboxylic acid-terminated polyethylene wax is UNICID® 550, available from Baker Petrolite, (USA). UNICID® 550 consists of 80% carboxylic acid functionality with the remainder a linear, low molecular weight polyethylene of a similar chain length, and an acid value of 72 mg KOH/g and melting point of about 101° C. Other suitable waxes have a structure  $\text{CH}_3-(\text{CH}_2)_n-\text{COOH}$ , such as hexadecanoic or palmitic acid with n=16, heptadecanoic or margaric or daturic acid with n=17, octadecanoic or stearic acid with n=18:0, eicosanoic or arachidic acid with n=20, docosanoic or behenic acid with n=22, tetracosanoic or lignoceric acid with n=24, hexacosanoic or cerotic acid with n=26, heptacosanoic or carboceric acid with n=27, octacosanoic or montanic acid with n=28, triacontanoic or melissic acid with n=30, dotriacontanoic or lacceroic acid with n=32, tritriacontanoic or ceromelissic or psyllic acid, with n=33, tetracontanoic or geddic acid with n=34, pentatriacontanoic or ceroplastic acid with n=35.

Suitable examples of amide waxes, such as aliphatic polar amide functionalized waxes, include, but are not limited to, stearamides, lauramides, palmitamides, behenamides, oleamides, erucamides, recinoleamides, mixtures thereof, and the like. Specific examples of suitable aliphatic polar amide functionalized waxes include, but are not limited to, stearyl stearamide, behenyl behenamide, stearyl behenamide, behenyl stearamide, oleyl oleamide, oleyl stearamide, stearyl oleamide, stearyl erucamide, oleyl palmitamide; methylol amide such as methylol stearamide or methylol behenamide, mixtures thereof, and the like. For example, a particularly suitable aliphatic polar amide functionalized wax is the stearyl stearamide wax KEMAMIDE® S-180, available from Witco, USA. Other types of nitrogen containing functional group waxes suitable for use in the hybrid wax system include amines, imides and quaternary amines, such as those available as JONCRYL® waxes from Johnson Diversey Inc.

Suitable examples of aliphatic waxes consisting of esters of hydroxylated unsaturated fatty acids, are those having a carbon chain length of from about 8 or less to about 20 or more or about 30 or more. For the aliphatic waxes consisting of esters of hydroxylated unsaturated fatty acids, any suitable chain length can be employed, so long as the functionality remains present and effective. In one particular embodiment, for example, the aliphatic waxes consisting of esters of hydroxylated unsaturated fatty acids have a chain length of for example from about 10 to about 16. For example, suitable in embodiments are those having a carbon chain length of approximately 12 units, such as from about 11 to about 13. Examples of such waxes include, but are not limited to, Carnauba wax and the like. For example, a particularly suitable crystalline aliphatic waxes consisting of esters of hydroxylated unsaturated fatty acids is RC-160 Carnauba wax, available from Toa Kasei, Japan.

Suitable examples of high acid waxes are acid waxes having a high acid content of, for example, greater than about 50% acid functionalized. Suitable high acid waxes are linear long chain aliphatic high acid waxes where a long

chain is a chain with 16 or more  $\text{CH}_2$  units. Linear, saturated, aliphatic waxes, such as having an end-functionalized carboxylic acid, are particularly suitable. Also suitable are high acid waxes with acid content of greater than about 50 mg 5 KOH/g. In embodiments, the high acid wax can be a montan wax, n-octacosanoic acid,  $\text{CH}_3(\text{CH}_2)_{26}-\text{COOH}$ , about 100% acid functionalized. Examples of such suitable montan waxes include, but are not limited to, Licowax® S, manufactured by Clariant, GmbH (Germany) with an acid 10 value of 127 to 160 mg KOH/g, Licowax® SW with acid value of 115-135, Licowax® UL with an acid value of 100-115 mg KOH/g and Licowax® X101 with acid value 15 130-150. Other suitable high acid waxes include partly esterified montanic acid waxes, where some of the acid 20 termination have been esterified, such as Licowax® U with an acid value of 72-92 mg KOH/g. Such high acid waxes are desired, in embodiments, because it has been found that they provide adequate charge stability to the toner composition, 25 since most emulsion/aggregation toner compositions have a high acid content (due to their constituent resin materials) and thus a resultant negative charge.

Microcrystalline waxes are derived from the distillation of crude oil. Microcrystalline waxes have molecular weights of about 500-675 g/m and melting points of about 73° C. to 94° 25 C. The waxes are highly branched and have smaller crystals. The typical microcrystalline wax crystal structure is small and thin, making the microcrystalline waxes tougher and more flexible and having higher tensile strengths and melting points than paraffin waxes. Variations in crystallinity, 30 amorphous material and molecular weight are responsible for the wide range of properties found in microcrystalline waxes. Examples of such suitable microcrystalline waxes include, but are not limited to, Michem Lube 124®, manufactured by Michelman Inc., Bareo High Melt Crystalline 35 Wax® and Bareo Flexible Microcrystalline Wax®, manufactured by Baker Petrolite, HP Wax 3040®, HP Wax 4076®, HP Wax 9508® manufactured by Hase Petroleum Wax Co., and the like.

Paraffin waxes are composed of straight-chained hydro- 40 carbon molecules originating from crude petroleum. The composition and properties of wax can be controlled through the refining process. Due to differences in the refining processes from manufacturers, waxes can vary. Some of the main grades of paraffin wax are fully refined, semi-refined, 45 and scale, depending upon the degree to which entrapped oil has been removed during refining. Color analysis can be used to differentiate these grades. Fully refined paraffins have less than 0.5% oil and are white and odorless. These materials are hard materials with melting points from 48 to 50 74 C. Semi-refined paraffin waxes contain more oil—0.5% to 1% making them softer and lighter-colored with a slight odor. Scale waxes are white or yellow soft materials with 1 to 3% oil content. The most refined grade of paraffin tends to be the glossiest. Examples of such suitable paraffin waxes 55 and paraffin wax mixtures include, but are not limited to, Michem Lube 723®, Michem Lube 743®, Michem Lube 693®, Michem Lube 180® (Carnauba and paraffin wax mixture), Michem Lube 182® (Carnauba and paraffin wax mixture) AOC PM30®, AOC PM53® manufactured by 60 Asheville Oil Company, and the like.

Fischer-Tropsch waxes are polymethylenes, synthetic hydrocarbons polymerized from natural gas (coal gasification). These waxes have molecular weights of about 300-1400 g/mole, and melt points of about 99° C., and provide 65 block, rub and scuff resistance. Fischer-Tropsch waxes are comprised of 90-95% normal paraffins, with the remainder being terminally branched tertiary and methyl hydrocarbons.

Fischer-Tropsch synthesis is the polymerization of carbon monoxide in the presence of hydrogen, using high pressure and unique catalysts to produce hydrocarbons. The process produces a distribution of chain lengths, which align with downstream products of fuel, lubricants and waxes. The product result depends on the catalyst, the process operation conditions (temperature, pressure, and residence time), and the distillation used to separate the hydrocarbons. Examples of such suitable Fischer-Tropsch waxes include, but are not limited to, BARECO® PX-105 Polymer, Michem Emulsion 64540® and Michem Emulsion® 98040M1, and the like.

Amine functionalized silicone waxes behave like typical hydrocarbon waxes in that they undergo a phase change from a solid to a viscous liquid over some well-defined temperature range. Examples of such suitable amine functionalized silicone waxes include, but are not limited to, GP61®, GP628®, GP7104®, GP7105, produced by Genesee Polymers Corporation, and the like. An exemplary structure of an amine functionalized silicone wax has the following structure:



where n and m represent the number of respective repeating units, and can generally range from about 1 or 2 to about 20 or 40 or more.

Silicone waxes behave like typical hydrocarbon waxes in that they undergo a phase change from a solid to a viscous liquid over some well-defined temperature range. Their structure is based on a combination of dimethyl silicone with organic wax side chains. Examples of such suitable silicone waxes include, but are not limited to, GP7104E®, GP7105E®, GP24LS®, GP7101, produced by Genesee Polymers Corporation, and the like.

Mercapto functionalized silicone waxes behave like typical hydrocarbon waxes in that they undergo a phase change from a solid to a viscous liquid over some well-defined temperature range. Examples of such suitable mercapto functionalized silicone waxes include, but are not limited to, GP77® and GP77E®, produced by Genesee Polymers Corporation, and the like. An exemplary structure of a Mercapto functionalized silicone wax has the following structure:



where n and m represent the number of respective repeating units, and can generally range from about 1 or 2 to about 20 or 40 or more.

Urethane waxes, also known as "isocyanate-derived waxes," as used in the present specification is defined as any crystalline or semi-crystalline waxy material derived from the reaction of a fatty isocyanate with a suitable nucleophile, or the reaction of a fatty nucleophile with a suitable isocy-

anate, or the reaction of a fatty nucleophile with a fatty isocyanate. Many such waxes are commonly available from commercial sources. Waxes found to be particularly useful for this purpose include, but are not limited to, N-octadecyclooctadecanamide, n-octadecyl isocyanate, reaction products of the following combinations: Tetradecanol, reaction products with polyisocyanates, Dodecanol, reaction products with polyisocyanates, Octanol, reaction products with polyisocyanates, Hexadecanol, reaction products with polyisocyanates, Docosanol, reaction products with polyisocyanates, Pentanol, reaction products with polyisocyanates, Decanol, reaction products with polyisocyanates, and the like.

Polyester waxes are made of ethylene glycol diesters or triesters of long-chain fatty acids (C18-C36). Their melting points range between about 60-75° C. and can be used to add stiffness and crystallinity. Polyester waxes are made to provide different physical properties. Straight chain esters, such as cetyl palmitate and cetylstearyl stearate, are solid at room temperature. Branched chain esters, such as isopropyl myristate or cetylstearyl ethylhexanoate, provide good spreading properties. These waxes may be selected from among any of the low melting point hydrophobic semi-crystalline polyester waxes evidencing a weight average molecular weight of from about 5,000 to about 80,000 and having a melting temperature within the range of about 55° C.-120° C. Many such waxes are commonly available from commercial sources. Waxes found to be particularly useful for this purpose include both aliphatic and aromatic semi-crystalline polyesters. The aliphatic semi-crystalline polyester waxes include: poly(butylene adipate), poly(hexamethylene sebacate), poly(decamethylene sebacate), and poly[hexamethylene-co-tetramethylene (80/20) cyclohexane dicarboxylate]. The semi-crystalline aromatic waxes include: poly[hexamethylene terephthalate-co-succinate (70/30)], poly[hexamethylene-co-tetramethylene (80/20)-terephthalate-co-isophthalate (80/20)], poly[hexamethylene-co-tetramethylene (80/20)-naphthonate-co-isophthalate (80/20)], poly[hexamethylene-co-2,2-dimethyl propylene (80/20)-terephthalate], and poly[hexamethylene-co-2,2-dimethylpropylene (80/20) naphthonate].

To incorporate the waxes into the toner, it is preferable for the waxes to be in the form of one or more aqueous emulsions or dispersions of solid wax in water, where the solid wax particle size is usually in the range of from about 100 to about 500 nm.

The toners may contain from, for example, about 3 to about 15% by weight of the toner, on a dry basis, of the hybrid wax system. For example, the toners contain from about 5 to about 11% by weight of the hybrid wax system.

In addition, the toners of the present disclosure may also optionally contain a coagulant and a flow agent such as colloidal silica. Suitable optional coagulants include any coagulant known or used in the art, including the well known coagulants polyaluminum chloride (PAC) and/or polyaluminum sulfosilicate (PASS). One suitable coagulant is polyaluminum chloride. The coagulant is present in the toner particles, exclusive of external additives and on a dry weight basis, in amounts of from 0 to about 3% by weight of the toner particles, such as from about greater than 0 to about 2% by weight of the toner particles. The flow agent, if present, may be any colloidal silica such as SNOWTEX OL colloidal silica, SNOWTEX OS colloidal silica, and/or mixtures thereof. The colloidal silica is present in the toner particles, exclusive of external additives and on a dry weight basis, in amounts of from 0 to about 15% by weight of the

## 11

toner particles, such as from about greater than 0 to about 10% by weight of the toner particles.

The toner may also include additional known positive or negative charge additives in effective suitable amounts of, for example, from about 0.1 to about 5 weight percent of the toner, such as quaternary ammonium compounds inclusive of alkyl pyridinium halides, bisulfates, organic sulfate and sulfonate compositions such as disclosed in U.S. Pat. No. 4,338,390, cetyl pyridinium tetrafluoroborates, distearyl dimethyl ammonium methyl sulfate, aluminum salts or complexes, and the like.

Also, in preparing the toner by the emulsion aggregation procedure, one or more surfactants may be used in the process. Suitable surfactants include anionic, cationic and nonionic surfactants.

Anionic surfactants include sodium dodecylsulfate (SDS), sodium dodecyl benzene sulfonate, sodium dodecyl-naphthalene sulfate, dialkyl benzenealkyl, sulfates and sulfonates, abitic acid, and the NEOGEN brand of anionic surfactants. An example of a suitable anionic surfactant is NEOGEN RK available from Daiichi Kogyo Seiyaku Co. Ltd., or TAYCA POWER BN2060 from Tayca Corporation (Japan), which consists primarily of branched sodium dodecyl benzene sulphonate.

Examples of cationic surfactants include dialkyl benzene alkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C<sub>12</sub>, C<sub>15</sub>, C<sub>17</sub> trimethyl ammonium bromides, halide salts of quaternized polyoxyethylalkylamines, dodecyl benzyl triethyl ammonium chloride, MIRAPOL and ALKAQUAT available from Alkaril Chemical Company, SANISOL (benzalkonium chloride), available from Kao Chemicals, and the like. An example of a suitable cationic surfactant is SANISOL B-50 available from Kao Corp., which consists primarily of benzyl dimethyl alkonium chloride.

Examples of nonionic surfactants include polyvinyl alcohol, polyacrylic acid, methalose, methyl cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxy poly(ethyleneoxy) ethanol, available from Rhone-Poulenc Inc. as IGEPAL CA-210, IGEPAL CA-520, IGEPAL CA-720, IGEPAL CO-890, IGEPAL CO-720, IGEPAL CO-290, IGEPAL CA-210, ANTAROX 890 and ANTAROX 897. An example of a suitable nonionic surfactant is ANTAROX 897 available from Rhone-Poulenc Inc., which consists primarily of alkyl phenol ethoxylate.

Any suitable emulsion aggregation procedure may be used in forming the emulsion aggregation toner particles without restriction. These procedures typically include the basic process steps of at least aggregating an emulsion containing binder, one or more colorants, optionally one or more surfactants, optionally a wax emulsion, optionally a coagulant and one or more additional optional additives to form aggregates, subsequently coalescing or fusing the aggregates, and then recovering, optionally washing and optionally drying the obtained emulsion aggregation toner particles.

An example emulsion/aggregation/coalescing process includes forming a mixture of latex binder, colorant dispersion, wax emulsion, optional coagulant and deionized water in a vessel. The mixture is then stirred using a homogenizer

## 12

until homogenized and then transferred to a reactor where the homogenized mixture is heated to a temperature of, for example, about 50° C. and held at such temperature for a period of time to permit aggregation of toner particles to the desired size. Once the desired size of aggregated toner particles is achieved, the pH of the mixture is adjusted in order to inhibit further toner aggregation. The toner particles are further heated to a temperature of, for example, about 90° C. and the pH lowered in order to enable the particles to coalesce and spherodize. The heater is then turned off and the reactor mixture allowed to cool to room temperature, at which point the aggregated and coalesced toner particles are recovered and optionally washed and dried.

Following coalescence and aggregation, the particles can be wet sieved through an orifice of a desired size in order to remove particles of too large a size, washed and treated to a desired pH, and then dried to a moisture content of, for example, less than 1% by weight.

The toner particles of the present disclosure can be made to have the following physical properties when no external additives are present on the toner particles.

The toner particles can have a surface area, as measured by the well known BET method, of about 1.3 to about 6.5 m<sup>2</sup>/g. For example, for cyan, yellow and black toner particles, the BET surface area is less than 2 m<sup>2</sup>/g, such as from about 1.4 to about 1.8 m<sup>2</sup>/g, and for magenta toner, from about 1.4 to about 6.3 m<sup>2</sup>/g.

It is also desirable to control the toner particle size and limit the amount of both fine and coarse toner particles in the toner. In an embodiment, the toner particles have a very narrow particle size distribution with a lower number ratio geometric standard deviation (GSD) of approximately 1.15 to approximately 1.30, or approximately less than 1.25. The toner particles of the present disclosure also can have a size such that the upper geometric standard deviation (GSD) by volume is in the range of from about 1.15 to about 1.30, such as from about 1.18 to about 1.22, or less than 1.25. These GSD values for the toner particles of the present disclosure indicate that the toner particles are made to have a very narrow particle size distribution.

Shape factor is also an important control process parameter associated with the toner being able to achieve optimal machine performance. The toner particles can have a shape factor of about 105 to about 170, such as about 110 to about 160, SF1\*a. Scanning electron microscopy (SEM) is used to determine the shape factor analysis of the toners by SEM and image analysis (IA) is tested. The average particle shapes are quantified by employing the following shape factor (SF1\*a) formula: SF1\*a=100πd<sup>2</sup>/(4A), where A is the area of the particle and d is its major axis. A perfectly circular or spherical particle has a shape factor of exactly 100. The shape factor SF1\*a increases as the shape becomes more irregular or elongated in shape with a higher surface area. In addition to measuring shape factor SF, another metric to measure particle circularity is being used on a regular bases. This is a faster method to quantify the particle shape. The instrument used is an FPIA-2100 manufactured by Sysmex. For a completely circular sphere the circularity would be 1.000. The toner particles can have circularity of about 0.920 to 0.990 and, such as from about 0.940 to about 0.975.

In addition to the foregoing, the toner particles of the present disclosure also have the following rheological and flow properties. First, the toner particles can have the following molecular weight values, each as determined by gel permeation chromatography (GPC) as known in the art.

The binder of the toner particles can have a weight average molecular weight, Mw of from about 15,000 daltons to about 90,000 daltons.

Overall, the toner particles in embodiments have a weight average molecular weight (Mw) in the range of about 17,000 to about 60,000 daltons, a number average molecular weight (Mn) of about 9,000 to about 18,000 daltons, and a MWD of about 2.1 to about 10. MWD is a ratio of the Mw to Mn of the toner particles, and is a measure of the polydispersity, or width, of the polymer. For cyan and yellow toners, the toner particles in embodiments can exhibit a weight average molecular weight (Mw) of about 22,000 to about 38,000 daltons, a number average molecular weight (Mn) of about 9,000 to about 13,000 daltons, and a MWD of about 2.2 to about 10. For black and magenta, the toner particles in embodiments can exhibit a weight average molecular weight (Mw) of about 22,000 to about 38,000 daltons, a number average molecular weight (Mn) of about 9,000 to about 13,000 daltons, and a MWD of about 2.2 to about 10.

Further, the toners if desired can have a specified relationship between the molecular weight of the latex binder and the molecular weight of the toner particles obtained following the emulsion aggregation procedure. As understood in the art, the binder undergoes crosslinking during processing, and the extent of crosslinking can be controlled during the process. The relationship can best be seen with respect to the molecular peak values for the binder. Molecular peak is the value that represents the highest peak of the weight average molecular weight. In the present disclosure, the binder can have a molecular peak (Mp) in the range of from about 22,000 to about 30,000 daltons, such as from about 22,500 to about 29,000 daltons. The toner particles prepared from such binder also exhibit a high molecular peak, for example of about 23,000 to about 32,000, such as about 23,500 to about 31,500 daltons, indicating that the molecular peak is driven by the properties of the binder rather than another component such as the colorant.

Another property of the toners of the present disclosure is the cohesivity of the particles prior to inclusion of any external additives. The greater the cohesivity, the less the toner particles are able to flow. The cohesivity of the toner particles, prior to inclusion of any external additives, may be from, for example, about 55 to about 98% for all colors of the toner. Cohesivity was measured by placing a known mass of toner, two grams, on top of a set of three screens, for example with screen meshes of 53 microns, 45 microns, and 38 microns in order from top to bottom, and vibrating the screens and toner for a fixed time at a fixed vibration amplitude, for example for 90 seconds at a 1 millimeter vibration amplitude. A device to perform this measurement is a Hosokawa Powders Tester, available from Micron Powders Systems. The toner cohesion value is related to the amount of toner remaining on each of the screens at the end of the time, and is calculated by the formula: % cohesion=50\*A+30\*B+10\*C, where A, B and C are respectively the weight of the toner remaining on the 53 microns, 45 microns, and 38 microns screens, respectively. A cohesion value of 100% corresponds to all of the toner remaining on the top screen at the end of the vibration step and a cohesion value of zero corresponds to all of the toner passing through all three screens, that is, no toner remaining on any of the three screens at the end of the vibration step. The higher the cohesion value, the lesser the flowability of the toner.

Finally, the toner particles in embodiments have a bulk density of from about 0.22 to about 0.34 g/cc and a compressibility of from about 33 to about 51.

The toner particles can be blended with external additives following formation. Any suitable surface additives may be used in embodiments. Most suitable are one or more of SiO<sub>2</sub>, metal oxides such as, for example, TiO<sub>2</sub> and aluminum oxide, and a lubricating agent such as, for example, a metal salt of a fatty acid (e.g., zinc stearate (ZnSt), calcium stearate) or long chain alcohols such as UNILIN 700, as external surface additives. In general, silica is applied to the toner surface for toner flow, tribo enhancement, admix control, improved development and transfer stability and higher toner blocking temperature. TiO<sub>2</sub> is applied for improved relative humidity (RH) stability, tribo control and improved development and transfer stability. Zinc stearate is optionally also used as an external additive for the toners of the disclosure, the zinc stearate providing lubricating properties. Zinc stearate provides developer conductivity and tribo enhancement, both due to its lubricating nature. In addition, zinc stearate enables higher toner charge and charge stability by increasing the number of contacts between toner and carrier particles. Calcium stearate and magnesium stearate provide similar functions. In embodiments, a commercially available zinc stearate known as Zinc Stearate L, obtained from Ferro Corporation, can be used. The external surface additives can be used with or without a coating.

In embodiments, the toners contain from, for example, about 0.1 to about 5 weight percent titania, about 0.1 to about 8 weight percent silica and about 0.1 to about 4 weight percent zinc stearate.

The toner particles of the disclosure can optionally be formulated into a developer composition by mixing the toner particles with carrier particles. Illustrative examples of carrier particles that can be selected for mixing with the toner composition prepared in accordance with the present disclosure include those particles that are capable of triboelectrically obtaining a charge of opposite polarity to that of the toner particles. Accordingly, in one embodiment the carrier particles may be selected so as to be of a negative polarity in order that the toner particles that are positively charged will adhere to and surround the carrier particles. Illustrative examples of such carrier particles include iron, iron alloys, steel, nickel, iron ferrites, including ferrites that incorporate strontium, magnesium, manganese, copper, zinc, and the like, magnetites, and the like. Additionally, there can be selected as carrier particles nickel berry carriers as disclosed in U.S. Pat. No. 3,847,604, the entire disclosure of which is totally incorporated herein by reference, comprised of nodular carrier beads of nickel, characterized by surfaces of reoccurring recesses and protrusions thereby providing particles with a relatively large external area. Other carriers are disclosed in U.S. Pat. Nos. 4,937,166 and 4,935,326, the disclosures of which are totally incorporated herein by reference.

The selected carrier particles can be used with or without a coating, the coating generally being comprised of acrylic and methacrylic polymers, such as methyl methacrylate, acrylic and methacrylic copolymers with fluoropolymers or with monoalkyl or dialkylamines, fluoropolymers, polyolefins, polystyrenes, such as polyvinylidene fluoride resins, terpolymers of styrene, methyl methacrylate, and a silane, such as triethoxy silane, tetrafluoroethylenes, other known coatings and the like.

The carrier particles can be mixed with the toner particles in various suitable combinations. The toner concentration is usually about 2% to about 10% by weight of toner and about 90% to about 98% by weight of carrier. However, one skilled in the art will recognize that different toner and

carrier percentages may be used to achieve a developer composition with desired characteristics.

Toners of the present disclosure can be used in known electrostatographic imaging methods. Thus for example, the toners or developers of the disclosure can be charged, e.g., triboelectrically, and applied to an oppositely charged latent image on an imaging member such as a photoreceptor or ionographic receiver. The resultant toner image can then be transferred, either directly or via an intermediate transport member, to a support such as paper or a transparency sheet. The toner image can then be fused to the support by application of heat and/or pressure, for example with a heated fuser roll.

It is envisioned that the toners of the present disclosure may be used in any suitable procedure for forming an image with a toner, including in applications other than xerographic applications.

Specific embodiments of the disclosure will now be described in detail. These Examples are intended to be illustrative, and the disclosure is not limited to the materials, conditions, or process parameters set forth in these embodiments. All parts and percentages are by weight unless otherwise indicated.

#### EXAMPLES

##### Comparative Example 1

A conventional styrene/n-butyl acrylate emulsion/aggregation toner containing 9% by weight polyethylene wax (POLYWAX® 725) is prepared as follows.

Step 1: Preparation of Latex Emulsion A. A latex emulsion comprised of polymer particles generated from the semi-continuous emulsion polymerization of styrene, n-butyl acrylate and beta carboxy ethyl acrylate ( $\beta$ -CEA) is prepared as follows. This reaction formulation is prepared in a 2 liter Buchi reactor, which can be readily scaled-up to a 100 gallon scale or larger by adjusting the quantities of materials accordingly.

A surfactant solution consisting of 0.9 grams Dowfax 2A1 (anionic emulsifier) and 514 grams de-ionized water is prepared by mixing for 10 minutes in a stainless steel holding tank. The holding tank is then purged with nitrogen for 5 minutes before transferring into the reactor. The reactor is then continuously purged with nitrogen while being stirred at 300 RPM. The reactor is then heated up to 76° C. at a controlled rate and held constant. In a separate container, 8.1 grams of ammonium persulfate initiator is dissolved in 45 grams of de-ionized water. Also in a second separate container, the monomer emulsion is prepared in the following manner; 426.6 grams of styrene, 113.4 grams of n-butyl acrylate and 16.2 grams of  $\beta$ -CEA, 11.3 grams of 1-dodecanethiol, 1.89 grams of ADOD, 10.59 grams of Dowfax (anionic surfactant), and 257 grams of deionized water are mixed to form an emulsion. The ratio of styrene monomer to n-butyl acrylate monomer by weight is 79 to 21 percent. One percent of the above emulsion is then slowly fed into the reactor containing the aqueous surfactant phase at 76° C. to form the "seeds" while being purged with nitrogen. The initiator solution is then slowly charged into the reactor and after 20 minutes the rest of the emulsion is continuously fed in using metering pumps. Once all the monomer emulsion is charged into the main reactor, the temperature is held at 76° C. for an additional 2 hours to complete the reaction. Full cooling is then applied and the reactor temperature is reduced to 35° C. The product is collected into a holding tank after filtration through a 1 micron filter bag. After

drying a portion of the latex the molecular properties are measured to be  $M_w=24,751$ ,  $M_n=8,245$  and the onset  $T_g$  is 51.46° C. The average particle size of the latex as measured by Disc Centrifuge is 203 nanometers and residual monomer as measured by GC as <50 ppm for styrene and <100 ppm for n-butyl acrylate. This latex is used to prepare emulsion/aggregation toner particles as described below.

Step 2: Preparation of toner particles from Latex Emulsion A containing 9% POLYWAX® 725. Into a 4 liter glass reactor equipped with an overhead stirrer and heating mantle is dispersed 639.9 grams of the above Latex Emulsion A having a 41.76 percent solids content, 135.53 grams of POLYWAX® 725 dispersion having a solids content of 30.63 percent, 92.6 grams of a Blue Pigment PB15:3 dispersion having a solids content of 26.49 percent into 1462.9 grams of water with high shear stirring by means of a polytron. To this mixture is added 54 grams of a coagulant solution consisting of 10 weight percent poly(aluminium-chloride), PAC and 90 wt. % 0.02M  $HNO_3$  solution. The PAC solution is added drop-wise at low rpm and as the viscosity of the pigmented latex mixture increases the rpm of the polytron probe also increases to 5,000 rpm for a period of 2 minutes. This produces a flocculation or heterocoagulation of gelled particles consisting of nanometer sized latex particles, 9% wax and 5% pigment for the core of the particles. The pigmented latex/wax slurry is heated at a controlled rate of 0.5 C/minute up to approximately 52° C. and held at this temperature or slightly higher to grow the particles to approximately 5.0 microns. Once the average particle size of 5.0 microns is achieved, 308.9 grams of the Latex Emulsion A is then introduced into the reactor while stirring. After an additional 30 minutes to 1 hour the particle size measured is 5.7 microns with a GSD of 1.20. The pH of the resulting mixture is then adjusted from 2.0 to 7.0 with aqueous base solution of 4 percent sodium hydroxide and allowed to stir for an additional 15 minutes. Subsequently, the resulting mixture is heated to 93° C. at 1.0° C. per minute and the particle size measured is 5.98 microns with a GSD by volume of 1.22 and GSD by number of 1.22. The pH is then reduced to 5.5 using a 2.5 percent Nitric acid solution. The resultant mixture is then allowed to coalesce for 2 hrs at a temperature of 93° C. The morphology of the particles is smooth and "potato" shape. The final particle size after cooling but before washing is 5.98 microns with a GSD by volume of 1.21. The particles are washed 6 times, where the 1st wash is conducted at pH of 10 at 63° C., followed by 3 washes with deionized water at room temperature, one wash carried out at a pH of 4.0 at 40° C., and finally the last wash with deionized water at room temperature. The final average particle size of the dried particles is 5.77 microns with  $GSD_v=1.21$  and  $GSD_n=1.25$ . The glass transition temperature of this sample is measured by DSC and found to have  $T_g(\text{onset})=49.4^\circ C$ .

The particles are dried blended with a standard additive package consisting of RY50 from Nippon Aerosil, JMT2000 from Tayca, X-24 from Shin-Etsu, EA latex particles of 1-5 micron size, and Unilin wax particles from Baker-Petrolite to produce a free flowing toner. Then 805 grams of developer is prepared at 5% toner concentration by weight, using 76.5 grams of this toner and 773.5 grams of 35 micron Xerox DocuColor 2240 carrier. The developer is conditioned overnight in A-zone and C-zone. The developer is evaluated in an Imari-MF free belt nip fuser (FBNF) system operating at a process speed of 104 mm/sec.

The image gloss fusing results of the toner composition obtained on the Imari-MF FBNF fixture are provided in FIG. 1 and compared to other single wax containing toners using

the same Latex Emulsion A. This includes the toner composition of Comparative Example 2 (9% KEMAMIDE® S-180 wax), the toner composition of Comparative Example 3 (9% RC-160 Carnauba wax), the toner composition of Comparative Example 4 (9% POLYWAX® 850), the toner composition of Comparative Example 5 (9% LICOWAX® S) and the toner composition of Comparative Example 6 (9% UNICID® 550 wax) instead on POLYWAX® 725. Provided in FIG. 2 is the Stripping Force results for this set of 6 toners. The dashed line for Stripping force at 25 grams of force indicates the specification for an acceptable level of force. The desired level is to be below 25 grams of force (gf).

#### Comparative Example 2

A conventional styrene/n-butyl acrylate emulsion/aggregation toner containing 9% KEMAMIDE® S-180 wax is prepared as follows.

The Latex Emulsion A is used to prepare this toner composition. The synthesis of this latex is provided in Comparative Example 1, Step 1. The aggregation/coalescence procedure used to prepare this toner is similar to that provided in Comparative Example 1, Step 2, except the POLYWAX® 725 aqueous dispersion is replaced with the equivalent weight percent of KEMAMIDE® S-180 wax also in the aqueous dispersion form. The final average particle size of the dried particles is 5.91 microns with  $GSD_v=1.22$  and  $GSD_n=1.22$ . The glass transition temperature of this sample is measured by DSC and found to have  $Tg(onset)=45.8^\circ C$ .

The particles are dried blended with the above-described standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

#### Comparative Example 3

A conventional styrene/n-butyl acrylate emulsion/aggregation toner containing 9% RC-160 Carnauba Wax is prepared as follows.

The Latex Emulsion A is used to prepare this toner composition. The synthesis of this latex is provided in Comparative Example 1, Step 1. The aggregation/coalescence procedure used to prepare this toner is similar to that provided in Comparative Example 1, Step 2, except the POLYWAX® 725 aqueous dispersion is replaced with the equivalent weight percent of RC-160 Carnauba wax also in the aqueous dispersion form. The final average particle size of the dried particles is 6.06 microns with  $GSD_v=1.20$  and  $GSD_n=1.25$ . The glass transition temperature of this sample is measured by DSC and found to have  $Tg(onset)=43.4^\circ C$ .

The particles are dried blended with the above-described standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

#### Comparative Example 4

A conventional styrene/n-butyl acrylate emulsion/aggregation toner containing 9% by weight polyethylene wax (POLYWAX® 850) is prepared as follows.

The Latex Emulsion A is used to prepared this toner composition. The synthesis of this latex is provided in Comparative Example 1, Step 1. The aggregation/coalescence procedure used to prepare this toner is similar to that provided in Comparative Example 1, Step 2, except the POLYWAX® 725 aqueous dispersion is replaced with the equivalent weight percent of POLYWAX® 850 wax also in the aqueous dispersion form. The final average particle size of the dried particles is 6.21 microns with  $GSD_v=1.21$  and  $GSD_n=1.23$ . The glass transition temperature of this sample is measured by DSC and found to have  $Tg(onset)=49.9^\circ C$ .

The particles are dried blended with a second standard additive package consisting of RY50 from Nippon Aerosil, JMT3103 from Tayca, X-24 from Shin-Etsu to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 nm/sec.

#### Comparative Example 5

A conventional styrene/n-butyl acrylate emulsion/aggregation toner containing 9% LICOWAX® S is prepared as follows.

The Latex Emulsion A is used to prepared this toner composition. The synthesis of this latex is provided in Comparative Example 1, Step 1. The aggregation/coalescence procedure used to prepare this toner is similar to that provided in Comparative Example 1, Step 2, except the POLYWAX® 725 aqueous dispersion is replaced with the equivalent weight percent of LICOWAX® S also in the aqueous dispersion form. The final average particle size of the dried particles is 5.98 microns with  $GSD_v=1.21$  and  $GSD_n=1.37$ . The glass transition temperature of this sample is measured by DSC and found to have  $Tg(onset)=43.7^\circ C$ .

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

#### Comparative Example 6

A conventional styrene/n-butyl acrylate emulsion/aggregation toner containing 9% UNICID® 550 Wax is prepared as follows.

The Latex Emulsion A is used to prepared this toner composition. The synthesis of this latex is provided in Comparative Example 1, Step 1. The aggregation/coalescence procedure used to prepare this toner is similar to that provided in Comparative Example 1, Step 2, except the POLYWAX® 725 aqueous dispersion is replaced with the equivalent weight percent of UNICID® 550 wax also in the aqueous dispersion form. The final average particle size of the dried particles is 6.05 microns with  $GSD_v=1.20$  and  $GSD_n=1.22$ . The glass transition temperature of this sample is measured by DSC and found to have  $Tg(onset)=45.6^\circ C$ .

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

## Discussion of Comparative Examples

Illustrated in FIG. 1 is the fused image gloss of 6 toners (Comparative Examples 1-6) all containing different crystalline polymeric waxes at the same weight percent loading of the toner. The toner compositions of Comparative Examples 1 and 4 contain POLYWAX® 725 and POLYWAX® 850, respectively. The image gloss of the toner compositions of Comparative Examples 1 and 4 is significantly less than the other 4 toners containing gloss enhancement crystalline polymeric waxes LICOWAX® S, RC-160 Carnauba wax, KEMAMIDE® S180 and UNICID® 550. Demonstrated in FIG. 2 is the evaluation of Stripping Force as a function of fusing temperature. Toners requiring a stripping force of greater than 25 grams of force generally do not meet current specifications. Only the toners containing POLYWAX® 725 or POLYWAX® 850 demonstrate good stripping force performance. The other high gloss toners containing the gloss enhancing waxes have very high stripping force performance and thus, do not meet the requirement for some fusing systems. Therefore, the present disclosure is the combination of the good stripping force performing waxes; either POLYWAX® 725 or POLYWAX® 850 with the one other crystalline polymeric wax, such as the four gloss enhancing waxes; KEMAMIDE® S180 or RC-160 Carnauba or LICOWAX® S or UNICID® 550.

## Example 1

A control styrene/n-butyl acrylate emulsion/aggregation toner containing 9% POLYWAX® 725 and Silica is prepared as follows.

Into a 4 liter glass reactor equipped with an overhead stirrer and heating mantle is dispersed 235.0 grams of Emulsion Latex B prepared in a similar manor to Emulsion Latex A described above having a 41.40 percent solids content, 53.98 grams of POLYWAX® 725 dispersion having a solids content of 30.76 percent, 57.7 grams of a Blue Pigment PB15:3 dispersion having a solids content of 17.0 percent into 531.4 grams of water with high shear stirring by means of a polytron. To this mixture after stirring for 20 minutes is first added 17.14 grams of colloidal silica SNOWTEX OL and 25.71 grams of colloidal silica SNOWTEX OS blended with 10.80 grams of a coagulant solution consisting of 10 weight percent poly(aluminum chloride) (PAC) and 90 weight percent 0.02M HNO<sub>3</sub> solution. After the silica mixture is blended into the latex, wax and pigment mixture the remaining PAC solution is added drop-wise at low rpm consisting of 21.6 grams of a coagulant solution consisting of 10 weight percent poly(aluminum chloride) (PAC) and 90 wt. % 0.02M HNO<sub>3</sub> solution. As the viscosity of the pigmented latex mixture increases the rpm of the polytron probe also increases to 5,000 rpm for a period of 2 minutes. This produces a flocculation or heterocoagulation of gelled particles consisting of nanometer sized latex particles, 9% wax and 5% pigment for the core of the particles. The pigmented latex/wax slurry is heated at a controlled rate of 0.5 °C./minute up to approximately 51° C. and held at this temperature or slightly higher to grow the particles to approximately 5.0 microns. Once the average particle size of 5.0 microns is achieved, 124.1 grams of the Emulsion Latex B is then introduced into the reactor while stirring. After an additional 30 minutes to 1 hour the particle size measured is 6.38 microns with a GSD of 1.20. The pH of the resulting mixture is then adjusted from 2.0 to 6.5 with aqueous base solution of 4 percent sodium hydroxide and allowed to stir

for an additional 15 minutes. Subsequently, the resulting mixture is heated to 96° C. at 1.0° C. per minute and the particle size measured is 7.19 microns with a GSD by volume of 1.22 and GSD by number of 1.27. The pH is then reduced to 6.3 using a 2.5 percent Nitric acid solution. The resultant mixture is then allowed to coalesce for 5 hrs at a temperature of 96° C. The morphology of the particles is smooth and "potato" shape. The final particle size after cooling but before washing is 6.64 microns with a GSD by volume of 1.20. The particles are washed 6 times, where the 1st wash is conducted at pH of 10 at 63° C., followed by 3 washes with deionized water at room temperature, one wash carried out at a pH of 4.0 at 40° C., and finally the last wash with deionized water at room temperature. The final average particle size of the dried particles is 6.64 microns with GSD<sub>v</sub>=1.20 and GSD<sub>n</sub>=1.24. The glass transition temperature of this sample is measured by DSC and found to have Tg(onset)=49.3° C. The yield of dried particles is 157.2 grams and the measured circularity is 0.956.

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

## Example 2

30 A styrene/n-butyl acrylate emulsion/aggregation toner containing 9% POLYWAX® 725 plus 3% LICOWAX® S and no silica is prepared as follows.

35 Into a 4 liter glass reactor equipped with an overhead stirrer and heating mantle is dispersed 243.8 grams of Emulsion Latex B having a 41.40 percent solids content, 53.98 grams of POLYWAX® 725 dispersion having a solids content of 30.76 percent, 28.48 grams of LICOWAX® S dispersion having a solids content of 18.96 percent, 57.7 grams of a Blue Pigment PB15:3 dispersion having a solids content of 17.00 percent into 549.0 grams of water with high 40 shear stirring by means of a polytron. To this mixture is added 32.4 grams of a coagulant solution consisting of 10 weight percent poly(aluminumchloride) (PAC) and 90 wt. % 0.02M HNO<sub>3</sub> solution. The PAC solution is added drop-wise at low rpm and as the viscosity of the pigmented latex 45 mixture increases the rpm of the polytron probe also increases to 5,000 rpm for a period of 2 minutes. This produces a flocculation or heterocoagulation of gelled particles consisting of nanometer sized latex particles, 12% wax and 5% pigment for the core of the particles. The pigmented latex/wax slurry is heated at a controlled rate of 0.5° C./minute up to approximately 51° C. and held at this 50 temperature or slightly higher to grow the particles to approximately 5.0 microns. Once the average particle size of 5.0 microns is achieved, 124.1 grams of the Emulsion Latex B is then introduced into the reactor while stirring. After an additional 30 minutes to 1 hour the particle size measured is 5.51 microns with a GSD of 1.20. The pH of the resulting mixture is then adjusted from 2.0 to 6.5 with aqueous base 55 solution of 4 percent sodium hydroxide and allowed to stir for an additional 15 minutes. Subsequently, the resulting mixture is heated to 96° C. at 1.0° C. per minute and the particle size measured is 5.97 microns with a GSD by volume of 1.21 and GSD by number of 1.24. The pH is then 60 reduced to 6.3 using a 2.5 percent Nitric acid solution. The resultant mixture is then allowed to coalesce for 5 hrs at a temperature of 96° C. The morphology of the particles is 65

smooth and "potato" shape. The final particle size after cooling but before washing is 5.97 microns with a GSD by volume of 1.21. The particles are washed 6 times, where the 1st wash is conducted at pH of 10 at 63° C., followed by 3 washes with deionized water at room temperature, one wash carried out at a pH of 4.0 at 40° C., and finally the last wash with deionized water at room temperature. The final average particle size of the dried particles is 5.89 microns with  $GSD_v=1.20$  and  $GSD_n=1.24$ . The glass transition temperature of this sample is measured by DSC and found to have  $Tg(onset)=48.5^\circ C$ . The yield of dried particles is 140.1 grams. The measured circularity of these particles is 0.974.

The particles are dried blended with the above-described second standard additive package to produce a free flowing toner. Then 805 grams of developer are prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

#### Example 3

A styrene/n-butyl acrylate emulsion/aggregation toner containing 9% POLYWAX® 725 plus 6% LICOWAX® S and no silica is prepared as follows.

The procedure followed to prepare this toner is the same as Example 2 except the weight percent of the LICOWAX® S is increased from 3 percent to 6 percent, which results in a reduction of the core Emulsion Latex B of 3 percent. The final average particle size of the dried particles is 6.13 microns with  $GSD_v=1.22$  and  $GSD_n=1.25$ . The glass transition temperature of this sample is measured by DSC and found to have  $Tg(onset)=44.74^\circ C$ . The yield of dried particles is 161.2 grams. The measured circularity of these particles is 0.945.

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

#### Example 4

A styrene/n-butyl acrylate emulsion/aggregation toner containing 9% POLYWAX® 725 plus 3% LICOWAX® S and colloidal silica is prepared as follows.

Into a 4 liter glass reactor equipped with an overhead stirrer and heating mantle is dispersed 221.7 grams of Emulsion Latex B having a 41.40 percent solids content, 53.98 grams of POLYWAX® 725 dispersion having a solids content of 30.76 percent, 28.48 grams of LICOWAX® S dispersion having a solids content of 18.96 percent, 57.7 grams of a Blue Pigment PB15:3 dispersion having a solids content of 17.0 percent into 526.8 grams of water with high shear stirring by means of a polytron. To this mixture after stirring for 20 minutes is first added 17.14 grams of colloidal silica SNOWTEX OL and 25.71 grams of colloidal silica SNOWTEX OS blended with 10.80 grams of a coagulant solution consisting of 10 weight percent poly(aluminum chloride) (PAC) and 90 weight percent 0.02M  $HNO_3$  solution. After the silica mixture is blended into the latex, wax and pigment mixture the remaining PAC solution is added drop-wise at low rpm consisting of 21.6 grams of a coagulant solution consisting of 10 weight percent poly(aluminum chloride), PAC and 90 wt. % 0.02M  $HNO_3$  solution. As the

viscosity of the pigmented latex mixture increases the rpm of the polytron probe also increases to 5,000 rpm for a period of 2 minutes. This produces a flocculation or heterocoagulation of gelled particles consisting of nanometer sized latex particles, 12% wax and 5% pigment for the core of the particles. The pigmented latex/wax slurry is heated at a controlled rate of 0.5° C./minute up to approximately 51° C. and held at this temperature or slightly higher to grow the particles to approximately 5.0 microns. Once the average particle size of 5.0 microns is achieved, 124.1 grams of the Emulsion Latex B is then introduced into the reactor while stirring. After an additional 30 minutes to 1 hour the particle size measured is 5.81 microns with a GSD of 1.19. The pH of the resulting mixture is then adjusted from 2.0 to 6.5 with aqueous base solution of 4 percent sodium hydroxide and allowed to stir for an additional 15 minutes. Subsequently, the resulting mixture is heated to 96° C. at 1.0° C. per minute and the particle size measured is 6.30 microns with a GSD by volume of 1.22 and GSD by number of 1.25. The pH is then reduced to 6.3 using a 2.5 percent Nitric acid solution. The resultant mixture is then allowed to coalesce for 5 hrs at a temperature of 96° C. The morphology of the particles is smooth and "potato" shape. The final particle size after cooling but before washing is 6.20 microns with a GSD by volume of 1.20. The particles are washed 6 times, where the 1st wash is conducted at pH of 10 at 63° C., followed by 3 washes with deionized water at room temperature, one wash carried out at a pH of 4.0 at 40° C., and finally the last wash with deionized water at room temperature. The final average particle size of the dried particles is 6.21 microns with  $GSD_v=1.20$  and  $GSD_n=1.24$ . The glass transition temperature of this sample is measured by DSC and found to have  $Tg(onset)=45.97^\circ C$ . The yield of dried particles is 155.6 grams and the measured circularity was 0.940.

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

#### Example 5

A styrene/n-butyl acrylate emulsion/aggregation toner containing 9% POLYWAX® 725 plus 6% LICOWAX® S and colloidal silica is prepared as follows.

The procedure followed to prepare this toner is the same as Example 4 except the weight percent of the LICOWAX® S is increased from 3 percent to 6 percent, which results in a reduction of the core Emulsion Latex B of 3 percent. The final average particle size of the dried particles is 6.13 microns with  $GSD_v=1.20$  and  $GSD_n=1.28$ . The glass transition temperature of this sample is measured by DSC and found to have  $Tg(onset)=40.47^\circ C$ . The yield of dried particles is 138.1 grams. The measured circularity of these particles is 0.951.

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

Illustrated in FIGS. 3a and 3b are the fused image gloss values of the 5 toners described in Examples 1 through 5 at a monolayer Total Mass per unit Area (TMA) (0.40 mg/cm<sup>2</sup>) and a Process Black TMA (1.05 mg/cm<sup>2</sup>), respectively, on Lustro Gloss Coated Paper. All toners are made from the same Emulsion Latex B, and all contain 9% by weight of POLYWAX® 725. The toner composition of Example 1 is the control toner made with 5% Silica and no additional gloss enhancing wax. The gloss at the FBNF run temperature of 160° C. represents the typical gloss value achieved by this machine at the full color process speed of 104 mm/sec. For a monolayer (i.e. single color) image, this value is about 40 gu, while for a Process Black TMA, it is still only about 45 gu. It is desirable that the image gloss should be at least as high as the gloss of the paper substrate, which for Lustro Gloss paper is about 70 gu. The toner composition of Example 4 has the same formulation as Example 1, with the inclusion of 3% LICOWAX®-S. Its gloss value at 160° C. is about 15 gu higher than Example 1 at low TMA, and about 20 gu higher than Example 1 at high TMA. Example 5 has the same formulation as Example 1 with the inclusion of 6% of LICOWAX® S. Its gloss value at 160° C. is about 30 gu higher than Example 1 at low TMA, and about 40 gu higher than Example 1 at high TMA. This toner also achieves the target gloss level of  $\geq 70$  gu at 160° C. at both low and high TMA.

Silica is included in the formulation of Example 1 to increase the gloss level over that of a similar toner made without silica. However, silica introduces considerable expense and complication into the process of making EA toner. Note that the gloss of Example 2 made with 3% LICOWAX® S, but no silica has almost the same, or slightly higher gloss than the control toner of Example 1. Therefore, the inclusion of 3% LICOWAX® S more than compensates for the reduction in gloss due to the removal of silica from the formulation. Moreover, the gloss of Example 3 with 6% LICOWAX® S and no silica is almost the same as Example 5 (6% LICOWAX® S, with silica). Therefore, by using LICOWAX® S, it may be possible to reach the targeted high gloss levels, even without the use of silica in the formulation. Note also that none of the gloss curves terminate before the maximum FBNF temperature of 200° C., due to Hot Offset of the toner image, as was the case for the toner containing only 9% LICOWAX® S, and no POLYWAX® 725 wax (Comparative Example 5) as shown in FIG. 1.

Illustrated in FIG. 4 are the Stripping Force values for the same set of 5 toners described in Examples 1 through 5. The maximum Stripping Forces for all 5 toners are well below the specified maximum value of 25 gf. The Stripping Force values for all toners made with 9% POLYWAX® 725 wax with 3% or 6% LICOWAX® S, (with or without silica), are the same order of magnitude as that of the control toner, Example 1, made with only 9% POLYWAX® 725 and no LICOWAX® S. This is in contrast to the toner made with only 9% LICOWAX® S and no POLYWAX® 725 wax (Comparative Example 5, shown in FIG. 2, which has a minimum Stripping Force that is more than 3x greater than the targeted maximum Stripping Force. Therefore, by combining a gloss enhancing wax, such as LICOWAX® S, with a wax that gives good release, such as POLYWAX® 725, in the same toner the present disclosure achieves the stated goal of reaching the target high gloss level, with no reduction in Hot Offset Temperature and no significant increase in Stripping Force.

A styrene/n-butyl acrylate emulsion/aggregation toner containing 9% POLYWAX® 725 Plus 3% RC-160 Carnauba Wax and no silica is prepared as follows.

Into a 4 liter glass reactor equipped with an overhead stirrer and heating mantle is dispersed 243.8 grams of Emulsion Latex B having a 41.40 percent solids content, 53.98 grams of POLYWAX® 725 dispersion having a solids content of 30.76 percent, 29.57 grams of RC-160 Carnauba wax dispersion having a solids content of 18.26 percent, 57.7 grams of a Blue Pigment PB15:3 dispersion having a solids content of 17.00 percent into 549.0 grams of water with high shear stirring by means of a polytron. To this mixture is added 32.4 grams of a coagulant solution consisting of 10 weight percent poly(aluminumchloride) (PAC) and 90 wt. % 0.02M HNO<sub>3</sub> solution. The PAC solution is added drop-wise at low rpm and as the viscosity of the pigmented latex mixture increases the rpm of the polytron probe also increases to 5,000 rpm for a period of 2 minutes. This produces a flocculation or heterocoagulation of gelled particles consisting of nanometer sized latex particles, 12% wax and 5% pigment for the core of the particles. The pigmented latex/wax slurry is heated at a controlled rate of 0.5° C./minute up to approximately 51° C. and held at this temperature or slightly higher to grow the particles to approximately 5.0 microns. Once the average particle size of 5.0 microns is achieved, 124.1 grams of Emulsion Latex B is then introduced into the reactor while stirring. After an additional 30 minutes to 1 hour the particle size measured is 6.85 microns with a GSD of 1.20. The pH of the resulting mixture is then adjusted from 2.0 to 6.5 with aqueous base solution of 4 percent sodium hydroxide and allowed to stir for an additional 15 minutes. Subsequently, the resulting mixture is heated to 96° C. at 1.0° C. per minute and the particle size measured is 7.10 microns with a GSD by volume of 1.19 and GSD by number of 1.25. The pH is then reduced to 6.3 using a 2.5 percent Nitric acid solution. The resultant mixture is then allowed to coalesce for 5 hrs at a temperature of 96° C. The morphology of the particles is smooth and "potato" shape. The final particle size after cooling but before washing is 5.97 microns with a GSD by volume of 1.21. The particles are washed 6 times, where the 1st wash is conducted at pH of 10 at 63° C., followed by 3 washes with deionized water at room temperature, one wash carried out at a pH of 4.0 at 40° C., and finally the last wash with deionized water at room temperature. The final average particle size of the dried particles is 7.00 microns with GSD<sub>v</sub>=1.19 and GSD<sub>n</sub>=1.26. The glass transition temperature of this sample is measured by DSC and found to have Tg(onset)=46.36° C. The yield of dried particles is 155.3 grams. The measured circularity of these particles is 0.939.

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

A styrene/n-butyl acrylate emulsion/aggregation toner containing 9% POLYWAX® 725 Plus 6% RC-160 Carnauba Wax and no silica is prepared as follows.

The procedure followed to prepare this toner is the same as Example 6 except the weight percent of the RC-160

## 25

Carnauba wax is increased from 3 percent to 6 percent, which results in a reduction of the core Emulsion Latex B of 3 percent. The final average particle size of the dried particles is 5.89 microns with  $GSD_v=1.19$  and  $GSD_n=1.24$ . The glass transition temperature of this sample is measured by DSC and found to have  $Tg(onset)=43.61^\circ C$ . The yield of dried particles is 137.8 grams. The measured circularity of these particles is 0.954.

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

## Example 8

A styrene/n-butyl acrylate emulsion/aggregation toner containing 9% POLYWAX® 725 Plus 3% RC-160 Carnauba Wax and colloidal silica is prepared as follows.

Into a 4 liter glass reactor equipped with an overhead stirrer and heating mantle is dispersed 221.7 grams of Emulsion Latex B having a 41.40 percent solids content, 53.98 grams of POLYWAX® 725 dispersion having a solids content of 30.76 percent, 30.31 grams of RC-160 Carnauba wax dispersion having a solids content of 18.26 percent, 57.7 grams of a Blue Pigment PB15:3 dispersion having a solids content of 17.0 percent into 526.8 grams of water with high shear stirring by means of a polytron. To this mixture after stirring for 20 minutes is first added 17.14 grams of colloidal silica SNOWTEX OL and 25.71 grams of colloidal silica SNOWTEX OS blended with 10.80 grams of a coagulant solution consisting of 10 weight percent poly(aluminum chloride) (PAC) and 90 weight percent 0.02M  $HNO_3$  solution. After the silica mixture is blended into the latex, wax and pigment mixture the remaining PAC solution is added drop-wise at low rpm consisting of 21.6 grams of a coagulant solution consisting of 10 weight percent poly(aluminum chloride) (PAC) and 90 wt. % 0.02M  $HNO_3$  solution. As the viscosity of the pigmented latex mixture increases the rpm of the polytron probe also increases to 5,000 rpm for a period of 2 minutes. This produces a flocculation or heterocoagulation of gelled particles consisting of nanometer sized latex particles, 12% wax and 5% pigment for the core of the particles. The pigmented latex/wax slurry is heated at a controlled rate of  $0.5^\circ C./minute$  up to approximately  $51^\circ C.$  and held at this temperature or slightly higher to grow the particles to approximately 5.0 microns. Once the average particle size of 5.0 microns is achieved, 124.1 grams of the Emulsion Latex B is then introduced into the reactor while stirring. After an additional 30 minutes to 1 hour the particle size measured is 5.84 microns with a GSD of 1.18. The pH of the resulting mixture is then adjusted from 2.0 to 6.5 with aqueous base solution of 4 percent sodium hydroxide and allowed to stir for an additional 15 minutes. Subsequently, the resulting mixture is heated to  $96^\circ C.$  at  $1.0^\circ C.$  per minute and the particle size measured is 6.06 microns with a GSD by volume of 1.20 and GSD by number of 1.22. The pH is then reduced to 6.3 using a 2.5 percent Nitric acid solution. The resultant mixture is then allowed to coalesce for 5 hrs at a temperature of  $96^\circ C.$  The morphology of the particles is smooth and "potato" shape. The final particle size after cooling but before washing is 6.06 microns with a GSD by volume of 1.18. The particles are washed 6 times, where the 1st wash is conducted at pH of 10 at  $63^\circ C.$ , followed by 3 washes with deionized water at room temperature, one wash

## 26

carried out at a pH of 4.0 at  $40^\circ C.$ , and finally the last wash with deionized water at room temperature. The final average particle size of the dried particles is 5.97 microns with  $GSD_v=1.19$  and  $GSD_n=1.23$ . The glass transition temperature of this sample is measured by DSC and found to have  $Tg(onset)=45.96^\circ C$ . The yield of dried particles is 147.2 grams and the measured circularity is 0.958.

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

15

## Example 9

A styrene/n-butyl acrylate emulsion/aggregation toner containing 9% POLYWAX® 725 Plus 6% RC-160 Carnauba Wax and colloidal silica is prepared as follows.

The procedure followed to prepare this toner is the same as Example 8 except the weight percent of the RC-160 Carnauba wax is increased from 3 percent to 6 percent, which results in a reduction of the core Emulsion Latex B of 3 percent. The final average particle size of the dried particles is 7.38 microns with  $GSD_v=1.20$  and  $GSD_n=1.36$ . The glass transition temperature of this sample is measured by DSC and found to have  $Tg(onset)=45.08^\circ C$ . The yield of dried particles is 148.0 grams. The measured circularity of these particles is 0.930.

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

35

## Example 10

A styrene/n-butyl acrylate emulsion/aggregation toner containing 9% POLYWAX® 725 Plus 6% UNICID® 500 and colloidal silica is prepared as follows.

The procedure followed to prepare this toner is the same as Example 9 except the RC-160 Carnauba wax dispersion consisting of 18.26 percent solids content is replaced with UNICID® 550 wax dispersion consisting of 19.15 percent solids content. The final average particle size of the dried particles is 5.91 microns with  $GSD_v=1.21$  and  $GSD_n=1.27$ . The glass transition temperature of this sample is measured by DSC and found to have  $Tg(onset)=46.00^\circ C$ . The yield of dried particles is 148.5 grams.

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

60

## Example 11

A styrene/n-butyl acrylate emulsion/aggregation toner containing 9% POLYWAX® 725 Plus 6% KEMAMIDE® S1180 and colloidal silica is prepared as follows.

The procedure followed to prepare this toner is the same as Example 9 except the RC-160 Carnauba wax dispersion

65

27

consisting of 18.26 percent solids content is replaced with KEMAMIDE® S180 wax dispersion consisting of 19.15 percent solids content. The final average particle size of the dried particles is 8.00 microns with  $GSD_v=1.21$  and  $GSD_n=1.29$ . The yield of dried particles is 148.6 grams.

The particles are dried blended with the above-described second standard additive package to produce a free flowing toner. Then 805 grams of developer is prepared using 76.5 grams of this toner and 773.5 grams of 35 micron Xerox DocuColor 2240 carrier. The developer is evaluated in the Imari-MF free belt nip fuser (FBNF) system operating at a process speed of 104 mm/sec.

#### Comparative Example 7

A conventional sulfonated polyester emulsion/aggregation toner containing 9% by weight Michelman 156 Carnauba wax is prepared as follows.

Into a 2 liter glass reactor equipped with an overhead stirrer and heating bath is dispersed 1000 grams of a sulfonated polyester latex having a solids content of 12 percent, 14.63 grams of Michelman 156 Carnauba wax dispersion having a solids content of 30 percent, and 18 grams of a pigment dispersion having a solids content of 48.8 percent (Sun Flexiverse® Pigment Blue 15:3) into 200 grams of water with agitator stirring at 275 rpm. The reactor jacket temperature is set to 60° C. and the mixture is heated to 59° C. while mixing at 275 rpm. Once this temperature is reached, the flow incorporation of zinc acetate is started, using a 10 mL/min addition rate for 40 minutes, then reduced to 1 mL/min until completely used. After optimum particle growth (5.5-5.8 microns) is achieved, the mixture is quenched with deionized water cooled to 34-36° F. The slurry is then mixed and filter-washed four times and then dried in a freeze drier for 48 hours.

The final product is toner particles having a morphology of smooth and "potato" shaped particles.

#### Comparative Example 8

The process of Comparative Example 7 is repeated, except that POLYWAX® 725 is substituted for the carnauba wax. The final product is toner particles having a morphology of bumpy and "potato" shaped particles, where the bumps present on the particles are wax protrusions.

#### Comparative Example 9

The process of Comparative Example 7 is repeated, except that the carnauba wax is omitted, and no wax is substituted in its place. The final product is toner particles having a morphology of smooth and round particles.

#### Example 12

The process of Comparative Example 7 is repeated, except that a hybrid wax system of 3 parts Baker Petrolite P725 polyethylene wax and 1 part Michelman 156 Carnauba wax are mixed. The final product is toner particles having a morphology of bumpy and "potato" shaped particles, where the bumps present on the particles are wax protrusions.

#### Example 13

The process of Comparative Example 7 is repeated, except that a hybrid wax system of 1.5 parts Michelman 156 Carnauba wax and 1 part Baker Petrolite P725 polyethylene

28

wax. The final product is toner particles having a morphology of bumpy and "potato" shaped particles, where the bumps present on the particles are wax protrusions.

The hybrid wax systems examine ratio differences using the mixture of Carnauba and polyethylene wax. Compared to the controls, the lack of wax does not provide sufficient release, but gives a smooth surface appearance. The addition of only polyethylene wax creates more wax protrusions on the surface of the particle, diminishing flow and increasing particle adhesion. The addition of only Carnauba wax reduces surface wax protrusions but may be too low melting for adequate fusing performance. By hybridizing the system with both waxes, a particle with improved surface wax and release properties can be created.

#### Comparative Example 10

The process of Comparative Example 7 is repeated, except that a microcrystalline wax Michelman 124 is substituted for the carnauba wax. The final product is toner particles having a morphology of spherical shaped particles that are somewhat porous on their surface.

#### Example 14

The process of Comparative Example 10 is repeated, except that a hybrid wax system of Michelman 162, composed of a mixture of microcrystalline and Carnauba waxes, is used. The final product is toner particles having a morphology of bumpy and "potato" shaped particles, where the bumps present on the particles are wax protrusions. The particles also lack the porosity evident on the surface of the toner particles of Comparative Example 10. The Carnauba control toner particle compared to the Carnauba/Microcrystalline Toner shows that the surface morphology could be modified by the addition of another wax type to change particle morphology and improve particle behavior in its performance.

It will be appreciated that various of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims.

What is claimed is:

1. A toner comprising particles of a resin, an optional colorant, a hybrid wax system composed of at least a first wax and a second wax,

wherein the waxes in the hybrid wax system are independently selected from the group consisting of polyolefin waxes; paraffin waxes; Fischer-Tropsch waxes; amine-functionalized silicone waxes; silicone waxes; mercapto-functionalized silicone waxes; polyester waxes; urethane waxes; modified polyolefin waxes; amide waxes; aliphatic waxes consisting of esters of hydroxylated unsaturated fatty acids; high acid waxes; and microcrystalline waxes,

wherein at least one wax in the hybrid wax system is a crystalline polymeric wax, and

wherein said toner particles are prepared by an emulsion aggregation process.

## 29

2. A toner according to claim 1, wherein the first wax and the second wax are different waxes.

3. A toner according to claim 1, wherein the toner further comprises a third wax that is different from the first and second waxes.

4. A toner according to claim 1, wherein a weight ratio of the first wax to the second wax ranges from about 5:95 to about 95:5.

5. A toner according to claim 1, wherein at least one of the first wax and the second wax comprises a linear polyethylene crystalline wax.

6. A toner according to claim 1, wherein at least one of the first wax and the second wax comprises a polyolefin wax.

7. A toner according to claim 6, wherein the polyolefin wax is selected from the group consisting of linear polyethylene waxes, branched polyethylene waxes, linear polypropylene waxes, and branched polypropylene waxes.

8. A toner according to claim 1, wherein at least one of the first wax and the second wax comprises a modified polyolefin wax.

9. A toner according to claim 8, wherein the modified polyolefin wax is a carboxylic acid-terminated wax.

10. A toner comprising particles of a resin, an optional colorant, a first wax and a second wax,

wherein the first wax and the second wax are independently selected from the group consisting of polyolefin waxes; paraffin waxes; Fischer-Tropsch waxes; amine-functionalized silicone waxes; silicone waxes; mercapto-functionalized silicone waxes; polyester waxes; urethane waxes; modified polyolefin waxes; amide waxes; aliphatic waxes consisting of esters of hydroxylated unsaturated fatty acids; high acid waxes; and microcrystalline waxes,

wherein the first wax and the second wax are selected such that the first wax provides improved results to the toner in terms of a first property over the second wax, while the second wax provides improved results to the toner in terms of a second property over the first wax, wherein the first property and the second property are selected from the group consisting of particle shape, charging characteristics, fusing characteristics, gloss, stripping and offset properties, and

wherein said toner particles are prepared by an emulsion aggregation process.

11. A toner according to claim 1, wherein the emulsion aggregation process comprises:

shearing a first ionic surfactant with a wax emulsion comprising said first wax and said second wax, and a latex mixture comprising (a) a counterionic surfactant with a charge polarity of opposite sign to that of said first ionic surfactant, (b) a nonionic surfactant, (c) a resin, and (d) an optional colorant, thereby causing flocculation or heterocoagulation of formed particles of resin to form electrostatically bound aggregates;

heating the electrostatically bound aggregates to form aggregates of at least about 1 micron in average particle diameter.

## 30

12. A toner according to claim 1, wherein the emulsion aggregation process comprises:

preparing a colorant dispersion in a solvent, which dispersion comprises a colorant and a first ionic surfactant; shearing the colorant dispersion with a wax emulsion comprising said first wax and said second wax, and a latex mixture comprising (a) a counterionic surfactant with a charge polarity of opposite sign to that of said first ionic surfactant, (b) a nonionic surfactant, and (c) a resin, thereby causing flocculation or heterocoagulation of formed particles of colorant and resin to form electrostatically bound aggregates; and

heating the electrostatically bound aggregates to form aggregates of at least about 1 micron in average particle diameter.

13. A toner according to claim 1, wherein the emulsion aggregation process comprises:

shearing an ionic surfactant with a wax emulsion comprising said first wax and said second wax, and a latex mixture comprising (a) a flocculating agent, (b) a nonionic surfactant, and (c) a resin, thereby causing flocculation or heterocoagulation of formed particles of colorant and resin to form electrostatically bound aggregates;

heating the electrostatically bound aggregates to form aggregates of at least about 1 micron in average particle diameter.

14. A toner according to claim 1, wherein the emulsion aggregation process comprises:

preparing a colorant dispersion in a solvent, which dispersion comprises a colorant and an ionic surfactant; shearing the colorant dispersion with a wax dispersion comprising said first wax and said second wax, and a latex mixture comprising (a) a flocculating agent, (b) a nonionic surfactant, and (c) a resin, thereby causing flocculation or heterocoagulation of formed particles of colorant and resin to form electrostatically bound aggregates; and

heating the electrostatically bound aggregates to form aggregates of at least about 1 micron in average particle diameter.

15. A toner according to claim 1, wherein the emulsion aggregation process comprises:

preparing a colloidal solution comprising a resin, said first wax, said second wax and an optional colorant, and adding to the colloidal solution an aqueous solution containing a coalescence agent comprising an ionic metal salt to form toner particles.

16. A developer comprising:

the toner of claim 1, and

a carrier.

17. An electrographic image development device, comprising the toner of claim 1 in a housing, a charging station, an imaging station with which the housing is associated, and a transferring station.

\* \* \* \* \*